

# UNITED STATES PATENT OFFICE.

JOSEF RICHTER, OF GENEVA, SWITZERLAND.

## METHOD OF MANUFACTURING STAMPING OR PRINTING DIES OR PLATES OR BLOCKS.

1,132,384.

Specification of Letters Patent. Patented Mar. 16, 1915.

No Drawing.

Application filed May 29, 1911. Serial No. 630,114.

*To all whom it may concern:*

Be it known that I, JOSEF RICHTER, subject of the Republic of Switzerland, residing at 3 Quai du Montblanc, Geneva, Switzerland, have invented certain new and useful Improvements in Improved Methods of Manufacturing Stamping or Printing Dies or Plates or Blocks, of which the following is a specification.

10 The present invention relates to an improved method of manufacturing, stamping or printing dies or plates or blocks. It has been proposed to use celluloid for this purpose, but such plates or blocks are too hard 15 at the edges and wear off too easily. Further, they do not properly fit to the surface onto which they are applied, and on the slightest superheating, which is generally unavoidable, blisters are formed. Attempts 20 have also been made to employ acetyl cellulose. This was obtained from solutions in acetic ether, chloroform or acetone, but sheets of sufficient thickness for making deep impressions can not be obtained, even 25 if non-drying oils and phenol derivatives are added to the solutions. These oils cause blisters and the masses obtained from the solutions are sticky. Further, these masses only soften at a high temperature, and it is 30 therefore necessary to heat them to 120°-150° centigrade. At these temperatures the acetyl cellulose decomposes and it is difficult to handle the hot sheets, more especially because paper, fabrics, or other 35 foundations become carbonized thereby.

According to the present invention the above disadvantages are obviated by employing masses which consist of acetyl cellulose preferably soluble in acetone, prepared in various ways to yield a suitable product, such as by treatment of acetone-soluble acetyl cellulose with mixtures of non-solvents or of solvents and non-solvents, with or without the addition of camphor 45 or camphor substitutes, and filling materials. Or acetone-soluble acetyl cellulose may be treated with camphor or camphor substitutes in quantities not sufficient for dissolving the acetyl cellulose. The above 50 known methods of preparing such masses are not claimed. The invention is concerned with the production from them of printing-plates, which is rendered possible by their special properties, *i. e.*, their hardness when cold, their low melting point, and their capacity of yielding a sharp impression when

heated even up to the melting point. The process is described more fully below. It essentially consists in heating the material above the softening point before making the impression. For example, these masses are produced from acetone-soluble acetyl cellulose which has been treated with camphor or camphor substitutes and cut into blocks or mechanically rolled. These masses are distinguished by their extreme hardness and exceedingly low softening point. Their melting point is even lower than that of celluloid as they melt or soften at about 70° centigrade. Now, the surprising fact has 60 been discovered that if sheets of this material, which can be obtained in any desired thickness of 2-3 millimeters and more are brought quite to the melting point, good printing blocks can be produced, although 65 partial decomposition takes place with the formation of blisters. It is on this remarkable property that the invention depends. The material is heated over 50° and up to 70° centigrade, when it becomes highly 75 softened. When the male counterparts are 80 pressed into the matrix, the blisters absolutely disappear under the pressure, the surface becomes perfectly smooth, and the details of the design appear in extraordinary 85 fineness, and in a surprising shading off of the middle tones. These effects can not be 90 obtained with celluloid or with the masses obtained from solutions of acetyl cellulose in ether, chloroform or acetone. 95

This process is also applicable in making printing blocks of objects such as lace, fabrics, relief designs and the like. These objects can be readily pressed into the highly 100 softened, hot material, thus producing a block which is equal to those made by the expensive way of engraving, etching or wood-carving. Reliefs and printing blocks can then be produced in any desired number by pressing the perfectly cold matrix 105 against a very hot softened sheet of the material, when the two parts can be taken apart a very short time after effecting the impression without damage. It is remarkable that this result is obtained even though 110 the sheets are not necessarily different in composition and can have exactly the same melting point. A material can be used in which filling materials, such as mica and other suitable substances, are added to the acetyl cellulose mass in quantities of from 50% upward. Reliefs or the articles to be 115

5 molded themselves or the like can be pressed into such material, thus forming a matrix from which as many counterparts can be molded as desired: even if the same material is used for the male counterpart and the matrix, these do not stick together as is the case with celluloid.

10 It is a very important advantage of the present invention that no shrinkage or variation of dimensions occurs by the evaporation of solvents, which is of special importance for multicolor printing. The dies, blocks or plates are very cheap as compared with metal printing blocks, they can 15 be quickly produced, are impervious to shocks or mechanical damages during transport, and are not affected by atmospheric influences. They serve for replacing metal printing blocks or rollers, steel engravings, 20 zinc clichés, sets of stereotypes, as well as cardboard and powder matrices. The printing surfaces are also very suitable for rotary printing, as they easily attach themselves to the cylinder and the like.

25 What I claim as new and desire to secure by Letters Patent is:—

30 1. A method of making a printing plate consisting in forming from acetyl cellulose soluble in acetone and camphor substitutes a hard solid body or mass having very 35 slight plasticity, said acetone and camphor substitutes being used in quantities not sufficient for dissolving the acetyl cellulose, the materials and proportions being specially selected so as to give a body having a softening 40 point of over 60° and below 100° C., then heating the said hard solid body to a point above the point at which it becomes plastic and nearly to the point at which it is made pasty by said heating, and while so heated forming it into a printing plate.

45 2. A method of making a printing plate consisting in forming from acetyl cellulose soluble in acetone and camphor substitutes a hard solid body or mass having very 50 slight plasticity, said acetone and camphor substitutes being used in quantities not sufficient for dissolving the acetyl cellulose, the materials and proportions being specially selected, together with the addition of more

than 50 per cent. of filling materials, so as to give a body having a softening point of over 60° and below 100° C., then heating the said hard solid body to a point above the point at which it becomes plastic and nearly 55 to the point at which it is made pasty by said heating, and while so heated forming it into a printing plate.

3. A method of making a printing plate consisting in forming from acetyl cellulose 60 soluble in acetone and camphor substitutes a hard solid body or mass having very slight plasticity, said acetone and camphor substitutes being used in quantities not sufficient for dissolving the acetyl cellulose, the 65 materials and proportions being specially selected so as to give a body having a softening point of over 60° and below 100° C., then heating said hard solid body or mass to a point above the point at which it becomes plastic and nearly 70 to the point at which it is made pasty by said heating and while so heated subjecting it to pressure against an object adapted to mold it into the desired form.

4. A method of making a printing plate consisting in forming from acetyl cellulose soluble in acetone and camphor substitutes a hard solid body or mass having very slight plasticity, said acetone and camphor 80 substitutes being used in quantities not sufficient for dissolving the acetyl cellulose, the materials and proportions being specially selected, together with the addition of more than 50 per cent. of filling materials, so as 85 to give a body having a softening point of over 60° or below 100° C., then heating said hard solid body or mass to a point above the point at which it becomes plastic and nearly 90 to the point at which it is made pasty by said heating and while so heated subjecting it to pressure against an object to mold it into the desired form.

In testimony whereof I affix my signature in presence of two witnesses.

JOSEF RICHTER.

Witnesses:

E. LOTTI,  
T. STRAUSS.